

## UNITED STATES PATENT OFFICE

2,234,565

## MOISTUREPROOF COATING

Daniel D. Lanning, Kenmore, N. Y., assignor to  
 E. I. du Pont de Nemours & Company, Wilming-  
 ton, Del., a corporation of Delaware

No Drawing. Application September 8, 1937,  
 Serial No. 162,888

18 Claims. (Cl. 91—68)

This invention relates to the production of coated structures. More particularly, it relates to moistureproofing coating compositions containing a new type of slip agent and the use of such coating compositions in the production of thin non-fibrous transparent sheets and films suitable for wrapping tissue having a coating which is non-tacky, slippery and non-adherent at elevated temperatures.

10 Thin transparent sheets and films of non-fibrous cellulosic materials containing moistureproof coatings are well known as wrapping tissue. In general, the coatings of such sheets and films comprise a film-forming constituent such as a cellulose derivative or a resin, a moistureproofing agent such as a wax, a blending agent such as a resin, and a plasticizer. Such moistureproofing coating compositions and methods for compounding and applying the same are disclosed in detail in the U. S. Patent No. 1,737,187 to Charch and Prindle and French Patent No. 718,440 to Charch.

Difficulty has long been experienced in the handling and storing of such sheets and films because of their lack of slipperiness and adherence of contiguous sheets to each other. These difficulties are due to at least two factors. One factor is that some of the constituents of the moistureproofing composition may be inherently tacky. A second factor is that the surfaces of these sheets are so smooth that, when they lie in close juxtaposition, they have a tendency to exclude air from between them, thus causing a vacuum action which renders it very difficult to separate the sheets, and at the same time to increase the area of contact, thus increasing the coefficient of friction. This smoothness is not overcome and in fact is accentuated by the ordinary constituents of the moistureproofing composition, particularly the moistureproofing agent, since it apparently forms a smooth continuous phase in order to prevent the passage of moisture.

Furthermore, it has been observed that these difficulties are greatly augmented by a slight rise in temperature. A sheet which proves perfectly satisfactory as to surface conditions at ordinary room temperatures may become very tacky and unmanageable when stored in heated places or when subjected to abnormally high room temperatures. Similar conditions have been found to arise in the use of automatic wrapping machinery. As long as such wrapping tissue is manually applied to packages, a slight

degree of stickiness and frictional resistance, while an inconvenience, is of no considerable consequence. It becomes of extreme importance, however, when such adherence and frictional resistance is increased by the transmission of heat or the heat developed by friction in an automatic machine. It is found actually that a difference of 1° or 2° may even cause a sticking of the material to some part or other of the machine and completely foul its operation. Furthermore, due to the high speeds developed in such automatic machinery, normal adherence and frictional resistance, even of the same degree as can be tolerated in manual operation, are objectionable even in the absence of a temperature rise.

An attempt has been made to overcome the adhesive tendency inherent in these films by the use of a thin layer of talcum powder. This method has the disadvantage, however, that while it lessens the adhesion of the sheets, it stains the film.

It has been suggested to incorporate small amounts of finely divided, insoluble materials, such as kaolin, aluminum hydroxide, titanium oxide, etc. in the moistureproofing coating compositions which are to be applied to the film. Since this solid matter is in a very finely divided form and since the coating bath is of relatively high viscosity, it is possible to disperse these solid particles in the bath and apply evenly to the surface of the film. The presence of such solid matter produces numerous points of separation between contiguous sheets in stacked relation, or between the surface of the sheet and other smooth surfaces, and thus insures good surface slip. However, the introduction of insoluble matter into the bath composition has several disadvantages. For one thing, it is very difficult to adequately disperse such solid materials without prolonged stirring and agitation and the dispersion may not be stable over long periods of time or in all conditions of operation, so that pipe lines and apparatus may become clogged with sediment. Furthermore, it is not possible to filter the bath composition once the solid, insoluble material has been added, and filtration is often necessary for the production of coating baths of the highest quality.

Another film defect from the use of such solid insoluble slip agents used heretofore has been a lowering of the moistureproof quality which is perhaps caused by interference with the continuity of the wax surface.

5

10

15

20

25

30

35

40

45

50

55

It is therefore an object of the present invention to produce a moistureproofing coating composition in which all constituents are in solution and which contains a solvent soluble slip agent 5 which will be somewhat incompatible with the other constituents of the coating in its final dry state.

It is another object of this invention to produce a transparent, non-fibrous sheet or film 10 containing a moistureproofing coating comprising a solvent soluble slip agent, which sheet or film will be substantially non-adherent at elevated temperatures.

Other objects of the invention will appear 15 hereinafter.

The objects of the invention may, generally, be attained by the use of a moistureproofing coating composition containing a solvent soluble, double metallic carboxylate which will be completely soluble in the liquid composition but which will not be completely compatible with the other constituents of the composition in its final dry state and which will therefore be present in a distinct phase from that of the main body of the 25 coating.

Although any double metallic carboxylate can be used provided it has the above solubility and compatibility requirements, the following test sets forth a convenient method for determining 30 the requisite characteristics of the most useful substances:

First, test the solubility of the substance in toluene at room temperature, or approximately 25° C. To function as a slip agent in the sense 35 of this invention, it must be soluble to the extent of 1% or more. Second, place 0.5 gram of the material in a test tube, add 25 cc. of acetone, place a stopper in the tube and shake. In this test also the temperature of the solvent should 40 be approximately 25° C. To function as a slip agent, the material must be partially or completely insoluble. If it is completely soluble, it will not function as a slip agent.

It is desirable that the slip agents separating 45 in a distinct phase from the coating composition upon the removal of the solvent shall have approximately the same optical characteristics as the coating composition itself. It therefore should preferably be substantially colorless (or 50 at least colorless in the concentration present in the final film) and have approximately the same index of refraction as the coating composition, such that the resulting product will appear transparent. The materials of the present 55 invention are well suited for this purpose. The following examples which are to be considered illustrative and not limitative will assist in an understanding of the invention.

The solvent soluble slip agents of the present 60 invention should preferably have the characteristic of raising the "stick temperature" (defined in detail below) of the coating composition above 55° C.

For the purposes of comparison and definition, 65 the following test is used to determine the stick temperature: A web of the material to be tested is moved across a table top and below a brass block with a surface of contact measuring 3½ x 1¼ inches, and weighing 500 grams, at the 70 uniform rate of 2 meters per minute. The temperature of the brass is slowly raised at the rate of about 7° C. per minute, and the frictional drag upon the film observed. This frictional drag at low temperatures is about 50-100 grams; at some 75 elevated temperature it increases suddenly to

several thousand grams, and the temperature at which this occurs is taken as the stick temperature.

As the double metallic carboxylates there may be used a double metal salt of a single carboxylic acid, of which zinc-aluminum rosinate is an example, or a single metal salt of two carboxylic acids, such as the aluminum salt of rosin and modified rosin, the aluminum salt of Petrex resin and modified rosin and the aluminum salt of phthalic acid and benzoyl benzoic acid. Other combinations are possible, such as salts of two metals and two acids. Likewise, more than two metallic or acid radicals may be present in the compound. The term "double metallic carboxylate," unless otherwise modified, is understood to include all these varieties.

The double metallic carboxylate should preferably be so selected that one of the corresponding single salts is highly soluble in the solvents used, such as toluene and ethyl acetate, and therefore presumably highly compatible with the other solids of the coating composition. The other corresponding single salt, on the other hand, should be of limited solubility in such solvents, and therefore only slightly compatible with the other solids of the coating composition.

These salts may be prepared as follows: predetermined quantities of the carboxylic acid or acids are dissolved in ethyl alcohol. The solution is neutralized with sodium hydroxide and then poured into an aqueous solution of an inorganic salt of the metal or metals to be introduced. The precipitate is washed and dried in vacuo at 45° C.

The following table gives the compositions of coating baths containing salts of certain organic acids which have been found to give excellent surface conditions and transparency when applied to transparent regenerated cellulose film. 40 In each case the stick temperature, as above defined, will be found given.

Table

|                         | Example Number  |                 |                 |                 | 45 |
|-------------------------|-----------------|-----------------|-----------------|-----------------|----|
|                         | 1               | 2               | 3               | 4               |    |
|                         | Parts by weight | Parts by weight | Parts by weight | Parts by weight | 50 |
| Double metallic salt    | 8               | 4               | 6               | 1               |    |
| Nitrocellulose, 11.6% N | 52              | 52              | 52              | 51              |    |
| Modified rosin          | 7               | 11              | 9               | 15              |    |
| Paraffin wax            | 3               | 3               | 3               | 3               |    |
| Diethyl phthalate       | 15              | 15              | 15              | 15              |    |
| Dicyclohexyl phthalate  | 15              | 15              | 15              | 15              |    |
| Ethyl acetate           | 440             | 440             | 440             | 440             | 55 |
| Toluene                 | 271             | 271             | 271             | 271             |    |
| Ethyl alcohol           | 22              | 22              | 22              | 22              |    |
| Stick temperature, °C.  | 60              | 71              | 62              | 59              |    |

In the above table, the double metallic salt of Example 1 is aluminum rosinate modified rosinate; of Example 2, aluminum zinc rosinate; of Example 3, aluminum salt of Petrex acid and of modified rosin; of Example 4, aluminum phthalate benzoyl benzoate. In each case the amount of the negative radicals or, in the case of Example 2, of the positive radicals are equal to each other.

The material which is added as a slip agent to the coating composition may also contribute other valuable properties to the coating. For instance, it may contribute to the body of the coating and serve to a certain extent as a blending agent for the wax and the nitrocellulose. In other cases the slip agent added may aid in

softening and plasticizing the coating. Advantage may be taken of such properties to so modify the coating composition as to effect a saving in some of the other ingredients such as resin, 5 blending agent, and plasticizer.

The slip agents of the present invention may be incorporated by any suitable method, preferably by dissolving in a suitable solvent such as toluene and then incorporating the remaining 10 ingredients, including solvents, of the moisture-proofing composition. Alternatively, the slip agents of the present invention as well as previously known insoluble slip agents may be introduced by the following method:

15 Cellulose nitrate in any form such as powder, flake, fiber or the like, is immersed in an aqueous solution of certain water soluble salts, such as aluminum sulfate or zinc acetate. This is then followed by treatment with a solution such 20 as ammonium hydroxide or sodium abietate which precipitates an insoluble slip agent on the pyroxylin structure. The treated cellulose nitrate is dried or dehydrated with alcohol and used directly in preparing lacquer solutions. 25 The method is very effective in producing moistureproof lacquers for regenerated cellulose film exhibiting good slip properties.

Still another general method of introducing silicon containing slip agents is represented by 30 the following example. Silicon compounds, either organic such as ethyl silicate or inorganic such as silicon tetrachloride, which react with water or alcohol to precipitate silicic acid may be added to lacquers containing water and/or alcohol to 35 produce a finely divided dispersion of silicic acid or an intermediate product of hydrolysis which is effective in producing lacquers with good slip.

The slip agents of this invention must be completely soluble in the solvent mixtures of the coating compositions, although they need not be soluble in every individual solvent of the solvent mixture. For this purpose any of the usual solvents and solvent mixtures familiar to one skilled 40 in the art will serve. Generally speaking, the 45 solvent will contain a cellulose derivative solvent and a wax solvent as well as a solvent for the resin and optionally a diluent. It is apparent that the same solvent may serve for two or more constituents and indeed, it may be that the 50 cellulose derivative solvent will also be a wax solvent. The solvent mixture comprising 40-90% ethyl acetate, 10-50% toluene, and the balance 55 ethyl alcohol will usually be found to operate satisfactorily. Depending on the amount and nature of the cellulose derivative or of the wax, or of the slip agent, etc., the amount and nature of the respective solvents will vary. Satisfactory solvents for the specific compositions are illustrated in the accompanying examples.

50 In the preparation of a transparent, moisture-proof wrapping tissue a suitable wax-containing composition comprising a cellulose derivative and a solvent soluble slip agent may be applied to the desired base in accordance with the methods known to the art. The solvents may be removed, and the coated material subjected to an elevated 55 temperature at least equal to the melting point of the wax, whence a clear, transparent, moistureproof film may be obtained. The technique of this procedure is set forth in such patents as the Charch and Prindle Patent No. 1,737,187.

While this invention has been described in terms of a coating composition comprising a cellulose derivative and certain other constituents 75 applied to a base film of regenerated cellulose or

other materials, it will be understood that it is equally applicable to the preparation of self-sustaining films of cellulose derivatives which are formed by extrusion, or casting, or other means from a solution in which the desired slip 5 agent is more soluble than in the resulting film.

Moistureproofing coating compositions may be used on various non-fibrous, transparent base sheets including sheets or films of regenerated cellulose, whether they be made by the viscose 10 process, the cuprammonium process, or by any other manufacturing technique; cellulose ethers such as ethyl, benzyl or glycol cellulose; cellulose esters such as cellulose nitrate or cellulose acetate; lowly etherified or esterified materials such 15 as lowly etherified ethyl cellulose, lowly etherified benzyl cellulose or lowly etherified glycol cellulose, and lowly esterified cellulose nitrate or lowly esterified cellulose acetate; gelatin, casein, or the like.

In preparing moistureproofing coating compositions comprising solvent soluble slip agents, it has been found that the best results are obtained by limiting the relative amounts of the several constituents. The amount of film-forming 20 constituent, for example, may vary from 30-70% or more of the total solids although in most instances 50-60% is to be preferred.

The solvent soluble slip agent may be present 25 in amounts of the order of 1-40% of the total 30 solids, depending upon its compatibility with the rest of the constituents of the coating composition when in the final dry state. The amount of the solvent soluble slip agent used in a coating 35 composition must be such that it will be completely soluble in the liquid coating composition but will, after removal of the solvent, separate 40 at least partially from the main body of the coating. Preferably it should be present in such quantity that the separate phase will constitute 45 only a small proportion of the total coating, such as 5% or less.

The wax content of these moistureproofing 50 compositions may vary from 0.5%, or 1% to 10%, or more of the total solids content. Usually about 45 4% is satisfactory, although more or less may be found desirable for different purposes.

The amount of plasticizer may vary, of course, 55 from none at all up to about 40 or 50% of the solids content of the composition.

The amount of solvent or solvent mixture may 60 vary according to the composition and to the method of application, or purpose desired. The viscosity of the coating composition may be controlled by the amount or nature of the solvent and 65 may be adjusted easily to adapt the solution for coating by brushing, spraying, dipping or any other methods familiar to the art.

Where percentages and proportions of ingredients are referred to throughout the specification 70 and claims, they are intended to be percentages by weight, or parts by weight.

The term "modified rosin" as used throughout the present specification and claims is defined as the rosin described and claimed in U. S. Letters Patent to Morton, No. 2,017,866; that is to say, a rosin having a high melting point, a high molecular weight, and being materially de-colored. This modified rosin is characterized generally by properties similar to those of rosin, 75 but with the difference that it has a molecular weight within the range 5% to 400% greater than ordinary rosin in its pure state; that it has a melting point, as determined by the capillary tube method, above 85° C. and higher 75

than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid.

The term "Petrox" as used throughout the present specification and claims is defined as the terpinene maleic anhydride complex comprising essentially 3 - isopropyl - 6 - methyl-3:6-endo-ethylene-delta-4-tetrahydro phthalic anhydride (J. Ind. Eng. Chem. XXIX, 21) marketed as "Petrox" resin by the Hercules Powder Co. It has an acid number of approximately 530, a molecular weight of approximately 215, and a softening point of 40°-50° C.

The surface conditioning agent of the present invention, when incorporated in coating compositions for use with transparent, cellulosic wrapping tissue, has been found to give a product which is eminently suited for use upon automatic wrapping machinery. For such use it is necessary that the tightly wound rolls of material supplied for use upon such machines unwind and deliver the film very smoothly and evenly through the machine. Even though rolls of such material have been tightly wound and stored at relatively high temperatures, it is found that there will be absolutely no sticking between the surfaces of the film, allowing it to unroll with great ease and freedom from tears, marred surfaces and other blemishes. It is furthermore essential that such material will pass evenly and smoothly through the whole course of the wrapping machine without adherence to various portions of said machine. Very often, certain heated elements form a part of such machines, said elements generally being used for the formation of heat seal at a certain stage of the wrapping operation. Should the adjacent parts of the machine become warm by conduction or convection of said heating elements, serious trouble may result in the operation of the machine by sticking of the wrapping tissue to these surfaces. The present invention produces a wrapping tissue which is far less likely to adhere to such surfaces than wrapping tissues previously available.

50 Where the coated wrapping tissue is in the form of sheets, said sheets may be stacked and stored for long periods of time without any appearance of adhesion between the sheets so stacked. Such sheets may be readily separated and handled manually or by machinery.

The method and materials of this invention produce an improved surface without adversely affecting clarity to the extent encountered in the use of the previously known insoluble slip agents.

In coating compositions giving moistureproofness, this moistureproofness is not affected so much by the solvent soluble slip agent as with previous insoluble slip agents.

65 The method of the invention has the very important advantage of giving a more uniform distribution of the surface conditioning agent throughout the coating bath which results in a far more even distribution in the coating with 70 the elimination of certain optical defects in the transparent film. Furthermore, it is possible to filter and purify the bath just before application to the film, making possible a very high grade product. Such filtration is not possible 75 where the agent added is a dispersed solid so

that large, solid particles and impurities that might occur in the bath at its later stages of preparation would remain to give trouble in the coating machinery and final product.

Not only may the use of the material be more precisely and rigidly controlled, but the disadvantages incident to sedimentation when the prepared bath solution is stored for a period of time, or transferred through pipes and under conditions which might cause the flocculation and sedimentation of a solid constituent are avoided.

By incorporating the double salts of the present invention in the coating composition, it is possible to obtain good slip in the coated surface over a much wider range of salt concentration than if the single salts of the same metals and acids are used. In some cases, the corresponding single salts, for example, are of only limited solubility in the solvents used, so that only limited quantities can be used. In other cases, the single salts are so highly compatible with the solid constituents of the coating composition that it is necessary to use very large quantities.

Since many changes and modifications can obviously be made from the details of the above description without departing from the nature and spirit of the invention, it is to be understood that the invention is not to be limited except as set forth in the following claims.

I claim:

1. A moistureproofing coating composition containing, dissolved in an organic solvent, a film-forming ingredient, a wax moistureproofing agent and the aluminum salt of rosin and modified rosin, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, said salt being present in sufficient quantity to separate as a distinct phase after the removal of the solvent, but in insufficient quantity to substantially impair the transparency of the coating.

2. A moistureproofing coating composition containing, dissolved in an organic solvent, a film-forming ingredient, a wax moistureproofing agent and zinc aluminum rosinate, said rosinate being present in sufficient quantity to separate as a distinct phase after the removal of the solvent but in insufficient quantity to substantially impair the transparency of the coating.

3. The article of claim 1, in which the double metallic carboxylate is the aluminum salt of rosin and modified rosin, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower

than that of pure abietic acid; and that it has a molecular weight higher than that of pure abietic acid.

4. The article of claim 9 in which the double metallic carboxylate is zinc aluminum rosinate.

5. A thin, flexible, slippery, non-fibrous, trans-

parent sheet provided with a moistureproofing

coating, said coating containing 30%-70% of a

film-forming ingredient, 0.5%-10% of a wax

moistureproofing agent, and 1%-40% of a slip

agent, said slip agent being in a phase separate

from the main body of the coating and being

from the group consisting of the aluminum salt

of rosin and modified rosin, the aluminum salt

of Petrex acid and modified rosin, aluminum

salt of phthalic acid and benzoyl benzoic acid,

and zinc aluminum rosinate, and having a sol-

ubility of at least 1% in toluene at a tempera-

ture of 25° C., and 0.5 grams of said carboxylate,

and being at least partially insoluble in 25 cc.

acetone at a temperature of 25° C., said modified

rosin being characterized by properties of the

general nature of those of rosin, but with the

difference that it has a molecular weight with-

in the range 5% to 400% greater than ordi-

nary rosin in its pure state; that it has a melt-

ing point, as determined by the capillary tube

method, above 85° C. and higher than the melt-

ing point of pure abietic acid and of purified

rosin when in the resinous state; that it is sub-

stantially free from combined sulfur and hard-

ening substances held in combination; that it

has an iodine value lower than that of pure

abietic acid; and that it has a molecular weight

higher than that of pure abietic acid, and said

Petrex acid being a terpinene maleic anhydride

complex comprising essentially 3-isopropyl-6-

methyl-3:6-endo - ethylene - delta-4-tetrahydro

phthalic anhydride.

40. 6. A thin, flexible, slippery, non-fibrous, trans-

parent sheet provided with a moistureproofing

coating, said coating containing 30%-70% of a

film forming ingredient, 0.5%-10% of a wax

moistureproofing agent, and 1%-40% of the

aluminum salt of modified rosin and Petrex

acid, said aluminum salt constituting a slip

agent in a phase separate from the main body of

the coating, said aluminum salt having a sol-

ubility of at least 1% toluene at a temperature of

25° C., and 0.5 grams thereof being at least par-

tially insoluble in 25 cc. acetone at a tempera-

ture of 25° C., said modified rosin being char-

acterized by properties of the general nature of

those of rosin, but with the difference that it

has a molecular weight within the range 5% to

400% greater than ordinary rosin in its pure

state; that it has a melting point, as determined

by the capillary tube method, above 85° C. and

higher than the melting point of pure abietic

acid and of purified rosin when in the resinous

state; that it is substantially free from combined

sulfur and hardening substances held in combina-

tion; that it has an iodine value lower than that

of pure abietic acid; and that it has a molecular

weight higher than that of pure abietic acid, and

said Petrex acid being a terpinene maleic anhydride

complex comprising essentially 3-isopropyl-6-

methyl-3:6-endo - ethylene - delta-4-tetrahydro

phthalic anhydride.

70. 7. A thin, flexible, slippery, non-fibrous, trans-

parent sheet provided with a moistureproofing

coating containing a film-forming ingredient, a

wax moistureproofing agent, and as a slip agent,

in a phase separate from the main body of the

coating, an organic solvent-soluble double

metallic carboxylate in an amount not exceeding

5% of the coating, said carboxylate having a

solubility of at least 1% in toluene at a tempera-

5 metallic carboxylate, said carboxylate having a solubility of at least 1% in toluene at a temperature of 25° C., and 0.5 grams of said slip agent being at least partially insoluble in 25 cc. acetone at a temperature of 25° C., and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene - delta-4-tetrahydro phthalic anhydride, said slip agent being present in insufficient quantity to substantially impair the transparency of the sheet.

30. 8. A thin, flexible, slippery, non-fibrous, trans-

parent sheet provided with a moistureproofing

coating containing a film-forming ingredient, and a wax moistureproofing agent, and as a slip

agent, in a phase separate from the main body

35 of the coating, 1% to 40% of an organic solvent-

soluble double metallic carboxylate, said car-

boxylate having a solubility of at least 1% in

toluene at a temperature of 25° C.; and 0.5 grams

40 of said compound being at least partially in-

soluble in 25 cc. acetone at a temperature of

25° C., and being from the group consisting of

45 the aluminum salt of rosin and modified rosin,

the aluminum salt of Petrex acid and modified

rosin, aluminum salt of phthalic acid and benzoyl

benzoic acid, and zinc aluminum rosinate, said

modified rosin being characterized by proper-

50 ties of the general nature of those of rosin, but

with the difference that it has a molecular weight

55 within the range 5% to 400% greater than ordi-

nary rosin in its pure state; that it has a melt-

ing point, as determined by the capillary tube

60 method, above 85° C. and higher than the melt-

ing point of pure abietic acid and of purified

65 rosin when in the resinous state; that it is sub-

stantially free from combined sulfur and harden-

ing substances held in combination; that it has

70 an iodine value lower than that of pure abietic

acid; and that it has a molecular weight higher

75 than that of pure abietic acid, and said Petrex

acid being a terpinene maleic anhydride com-

plex comprising essentially 3-isopropyl-6-

methyl-3:6-endo-ethylene - delta-4-tetrahydro

80 phthalic anhydride, said compound being present

in insufficient quantity to substantially impair

85 the transparency of the sheet.

9. A thin, flexible, slippery, non-fibrous, trans-

parent sheet provided with a moistureproofing

coating containing a film-forming ingredient, a

wax moistureproofing agent, and as a slip agent,

95 in a phase separate from the main body of the

coating, an organic solvent-soluble double

metallic carboxylate in an amount not exceeding

100 5% of the coating, said carboxylate having a

solubility of at least 1% in toluene at a tempera-

ture of 25° C., and 0.5 grams of said carboxylate being at least partially insoluble in 25 cc. acetone at a temperature of 25° C., and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4-tetrahydro phthalic anhydride.

10. A moistureproofing coating composition containing, dissolved in an organic solvent, a film-forming ingredient, a wax moistureproofing agent and a double metallic carboxylate, said carboxylate having a solubility of at least 1% in toluene at a temperature of 25° C., and 0.5 grams of said carboxylate being at least partially insoluble in 25 cc. acetone at a temperature of 25° C., and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4-tetrahydro phthalic anhydride, said carboxylate being present in sufficient quantity to separate as a distinct phase after the removal of the solvent, but in insufficient quantity to substantially impair the transparency of the coating.

11. A moistureproofing coating composition containing, dissolved in an organic solvent, a film-forming ingredient, a wax moistureproofing agent and the aluminum salt of modified rosin and Petrex acid, the quantity of said salt being sufficient to separate as a distinct phase but insufficient to substantially impair the transparency of the coating after the removal of the solvent, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride

the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4-tetrahydro phthalic anhydride.

12. A moistureproofing coating composition containing, dissolved in an organic solvent, a film-forming ingredient, a wax moistureproofing agent and 1% to 40% (based on the solids content) of a double metallic carboxylate, said carboxylate having a solubility of at least 1% in toluene at a temperature of 25° C., and 0.5 grams of said carboxylate being at least partially insoluble in 25 cc. acetone at a temperature of 25° C., and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4-tetrahydro phthalic anhydride, said carboxylate being present in sufficient quantity to separate as a distinct phase after the removal of the solvent, but in insufficient quantity to substantially impair the transparency of the coating.

13. A moistureproofing coating composition containing, dissolved in an organic solvent, a film-forming ingredient, a wax moistureproofing agent and a double metallic carboxylate, said carboxylate having a solubility of at least 1% in toluene at a temperature of 25° C., and 0.5 grams of said carboxylate being at least partially insoluble in 25 cc. acetone at a temperature of 25° C., and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride

complex comprising essentially 3-isopropyl-6-methyl-3:6-endo-ethylene-delta - 4 - tetrahydro phthalic anhydride, said carboxylate being present in sufficient quantity to separate as a distinct phase after the removal of the solvent, but said distinct phase of the carboxylate not exceeding 5%.

14. The method of producing a thin, flexible, slippery, high-stick temperature, transparent, moistureproof sheet which comprises applying to a transparent, non-fibrous base sheet a moisture-proofing coating composition containing in solution 30%-70% of a film-forming ingredient, 0.5%-10% of a moistureproofing agent, and 1%-40% of a slip agent of the group consisting of the aluminum salt of rosin and modified rosin, the aluminum salt of Petrex acid and modified rosin, aluminum salt of phthalic acid and benzoyl benzoic acid, and zinc aluminum rosinate, and drying said coating composition whereby to cause said slip agent to separate as a distinct phase from the main body of the coating, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3 - isopropyl-6-methyl-3:6 - endo-ethylene-delta-4-tetrahydro phthalic anhydride.

15. The method of producing a thin, flexible, slippery, high-stick temperature, transparent, moistureproof sheet which comprises applying to a transparent, non-fibrous base sheet a moisture-proofing coating composition containing in solution a film-forming ingredient, a moistureproofing agent, and a double metallic carboxylate, said carboxylate being present in sufficient quantity to separate as a distinct phase after the removal of the solvent, but in insufficient quantity to substantially impair the transparency of the coating, and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4 - tetrahydro phthalic anhydride, and drying said coating composition whereby to cause said carboxylate to separate as a distinct phase from the main body of the coating in an amount not exceeding 5%.

said carboxylate to separate as a distinct phase from the main body of the coating.

16. The method of producing a thin, flexible, slippery, high-stick temperature, transparent, moistureproof sheet which comprises applying to a transparent, non-fibrous base sheet a moisture-proofing coating composition containing in solution 30%-70% of a film-forming ingredient, 0.5%-10% of a moistureproofing agent, and 1%-40% of the aluminum salt of modified rosin and Petrex acid, and drying said coating composition whereby to cause said aluminum salt to separate as a distinct phase from the main body of the coating, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4 - tetrahydro phthalic anhydride.

17. The method of producing a thin, flexible, slippery, high-stick temperature, transparent, moistureproof sheet which comprises applying to a transparent, non-fibrous base sheet a moisture-proofing coating composition containing in solution a film-forming ingredient, a moistureproofing agent and 1% to 40% (based on the solids content) of a double metallic carboxylate, said carboxylate being present in sufficient quantity to separate as a distinct phase after the removal of the solvent but in insufficient quantity to substantially impair the transparency of the coating, and being from the group consisting of the aluminum salt of rosin and modified rosin, the aluminum salt of Petrex acid and modified rosin, aluminum salt of phthalic acid and benzoyl benzoic acid, and zinc aluminum rosinate, said modified rosin being characterized by properties of the general nature of those of rosin, but with the difference that it has a molecular weight within the range 5% to 400% greater than ordinary rosin in its pure state; that it has a melting point, as determined by the capillary tube method, above 85° C. and higher than the melting point of pure abietic acid and of purified rosin when in the resinous state; that it is substantially free from combined sulfur and hardening substances held in combination; that it has an iodine value lower than that of pure abietic acid, and said Petrex acid being a terpinene maleic anhydride complex comprising essentially 3-isopropyl-6-methyl-3:6-endo-ethylene-delta-4 - tetrahydro phthalic anhydride, and drying said coating composition whereby to cause said carboxylate to separate as a distinct phase from the main body of the coating in an amount not exceeding 5%.

18. The article of claim 9 in which the double metallic carboxylate is the aluminum salt of modified rosin and of Petrex acid, said modified rosin being characterized by properties of the general nature of those of rosin, but with the difference that it has a molecular weight within the range 5% to 400% greater than ordinary rosin in 75

its pure state; that it has a melting point, as determined by the capillary tube method, above 85° C. and higher than the melting point of pure abietic acid and of purified rosin when in the 5 resinous state; that it is substantially free from combined sulfur and hardening substances held in combination; that it has an iodine value lower

than that of pure abietic acid; and that it has a molecular weight higher than that of pure abietic acid, and said Petrex acid being a terpinene maleic anhydride complex comprising essentially 3-isopropyl-6-methyl-3:6-endo-ethylene-delta-4- 5 tetrahydro phthalic anhydride.

DANIEL D. LANNING.